

## UNITED STATES PATENT OFFICE

2,421,622

## ALKYL CARBAMATES IN COLOR COMPOSITIONS

Roy Herman Kienle and Chester Albert Amick,  
Bound Brook, N. J., assignors to American Cyanamid Company, New York, N. Y., a corporation of Maine

No Drawing. Application July 1, 1943,  
Serial No. 493,129

12 Claims. (Cl. 8—70)

1

This invention relates to a new type of dyeing and printing assistant, dye compositions containing these assistants and products printed therefrom.

Use of printing-color pastes containing dyes, particularly in printing operations using vat dyes, is sufficiently well-known so that the procedure has become almost standardized. The actual color source may be either a dye paste or a dye powder. In addition to the real color, a dye paste usually contains agents to prevent drying-out, settling and/or freezing. Dye powders, not being subject to these difficulties, do not require these agents but they usually contain agents or are so processed as to promote dispersibility.

In either case, the dye paste or dye powder must be admixed with suitable thickener, usually a gum dispersion, to form a printing-color paste which is suitable for application. In the case of vat dyes, it is also necessary to add a reducing agent and usually an alkali. Because the color yield from printing-color pastes often decreases rapidly as the paste ages after being made up, these printing-color pastes are usually prepared by the fabric finishers just before they are to be used.

The printing-color pastes, however compounded, are then applied to textile, paper or other fabric materials for decorative or protective purposes. The printed pieces are dried, aged in a steam ager, treated with an oxidizing agent, rinsed and finally dried. Usually in processing textiles, the printed fabric also is soaped at or near the boil with about a 0.1% soap solution and again rinsed before the final drying operation.

In making up and applying printing-color pastes it has been found that a material suitable for use as a printing assistant is of advantage in obtaining maximum color yield. The exact way in which these materials act to produce an improved color yield in printing is not entirely understood. It is with these printing aids or assistants that the present invention is particularly concerned.

Although printing aids are desirable in the printing-color pastes, the exact point at which they are added may vary. Dye pastes may contain printing aids as one of their components and printing-color pastes made therefrom will obviously contain the printing assistant. Where a printing assistant is not present in the dye paste, it may be added at the time of making up the printing-color paste.

It is preferable, however, that the printing assistant be incorporated in the actual dye paste. Their addition at the proper point in the manu-

2

facture of the paste is not only easier, but in addition they are thus generally more uniformly dispersed throughout a printing-color paste made therefrom. As a result, the printing assistants usually operate more effectively when the printing-color paste is finally applied to the fabric.

It is only relatively recently that dye powders suitable for use in making up printing-color pastes have been available. Most of the printing aids previously used in dye pastes, being either liquid in form or extremely hydroscopic, can not be used with dye powders, the latter being necessarily limited to the use of dry solids. Nevertheless, it is desirable that printing assistants be incorporated in the powders at the time of manufacture for the same reasons which apply in the case of dye pastes.

Dye pastes containing various liquid printing assistants have been made. Among the liquid materials used are the alkylol amines, for example, triethanol amine; and/or polyhydric alcohols such as glycerine, glycol, diethylene glycol and the like. Various derivatives therefrom also have been tried. If a printing aid is to be incorporated in a dye powder, a solid printing aid is necessary. Examples of such solids which have been used in the past include the hydrochlorides of alkylol amines; silver salt (sodium anthraquinone beta-sulfonate); anthraquinone and certain metal salts such as those of cobalt and iron.

Unfortunately, most of these printing aids previously used are not as satisfactory as may be desired. Many of them will not in all cases produce the intensification of color for which they were intended. Others, such as the polyhydric alcohols, cause deterioration of the printing-color pastes so that marked variations in the strength of prints therefrom are observable even after the printing-color paste has been allowed to stand for only a relatively short time. Many of them are satisfactory with some colors but have an adverse effect on others, even to the extent of visibly altering the shade. None of them are suitable without modification for use both in paste and powder compositions.

There remains, therefore, a demand for suitable printing assistants which will produce a satisfactory color intensification and will not cause deterioration of the dyeing or printing composition on standing. Preferably also, the assistants should be useful both with dye pastes and dye powders and in addition should be readily available or cheaply and easily prepared. It is, therefore, the object of the present invention to pro-

vide a new type of printing assistant which possesses these desirable properties.

In general, the object of the present invention is accomplished by making use of a solid urethane. According to the present invention the expression "a urethane" is intended to include not only urethane itself, but also those solid alkyl carbamates which are the reaction products of a monohydric aliphatic alcohol and a urea or substituted urea, particularly the alkyl-substituted ureas. So far as the present invention is concerned the urethanes may be added to the printing-color pastes at any point in their compounding. They may be incorporated into the thickener; into the dye pastes or powders or may be blended into the printing-color paste when the latter composition is prepared. However, as pointed out above, it is preferable that they be incorporated in the dye paste or powder during their manufacture.

The use of this new class of printing assistants possesses a number of important advantages. Most of these products are dry powders but are soluble or dispersible in dye paste suspensions so that they may be used in all cases. They do not cause deterioration of the printing-color pastes on standing. They encourage the production of excellent color yields even under hot ageing conditions. Their use is simple since they may be employed as powders, as suspensions in water or as alcoholic solutions, producing excellent color yields whatever the mode of admixture.

In producing the alkyl carbamates of the present invention it is not necessary to limit the assistant to the reaction product of any particular monohydric alcohol. Substantially any monohydric aliphatic alcohol of from about three to twelve carbon atoms can be reacted with an urea or a substituted-urea to produce a carbamate useful according to the present invention. While the invention is not intended to be so limited, it has been found that the use of primary or secondary aliphatic alcohols having from about four to eight carbon atoms appear to give wholly satisfactory products. Excellent results have been obtained, for example, using the reaction product of butyl, ethylbutyl, or an octyl alcohol with urea and such substituted-ureas as methyl, ethyl, diethyl, di-n-butyl, ethyl nitroso and phenyl urea.

While the dye and printing paste compositions of the present invention are not limited to the use of any particular dyes or dye forms, they are especially suitable for use with vat-dyes in either paste or powder form. Particularly good results may be obtained using the vat-dye powders of high autodispersibility as set forth in Crossley et al., Reissue Patent No. 21,402, re-issued March 19, 1940. By combining the color materials of that patent into printing paste composition containing the assistants of the present invention, the full advantages of both may be gained with a resultant excellence of shade and sharpness of color.

Printing pastes made in this way have the particular advantage that the dyes remain in a highly dispersed state as individual particles rather than as dispersions of particle aggregates. In the present specification and claims, where highly-dispersed dyes are referred to, reference to pastes in which the dye particles are so dispersed is intended.

The invention will be more fully set forth in connection with the following examples which are intended to be illustrative only and not by

way of limitation. All parts are by weight unless otherwise noted.

*Example 1*

5 A paste was prepared by slurring 2,000 parts of 177 British gum (Stein Hall) in 5,000 parts of water and the mixture was heated with continuous stirring until the temperature reached about 185° F. Heating was continued for about 10 1½ hours after which 450 parts of powdered potassium carbonate and 450 parts of powdered sodium carbonate were added and the mixture stirred until the carbonates dissolved. Heating was discontinued but stirring was continued until 15 the temperature reached approximately 150° F. at which time 700 parts of sodium sulfoxylate formaldehyde were dissolved therein, 600 parts of glycerine were added and the paste bulked to about 10,000 parts. Stirring was continued until 20 the paste cooled to room temperature. In the succeeding examples this paste is referred to as Thickener A.

*Example 2*

25 720 parts of B-2 British gum and 720 parts of KAC-4 gum (Stein Hall) were added to 5600 parts of water and heated over a steam bath for approximately 1½ hours after the temperature reached about 185°-190° F. The source of heat was then removed but stirring was continued 30 until the temperature decreased to 130° F. at which time 1200 parts of potassium carbonate which had been previously dissolved in 1000 parts of water was added to the cooked gum. 1560 parts of sodium sulfoxylate formaldehyde were 35 dissolved in 1500 parts of water at a temperature of about 140° F. and added to the common mixture with stirring until the whole was thoroughly mixed. 360 parts of glycerine were added and after thorough stirring the whole was bulked to 40 about 12000 parts. In the succeeding examples this is referred to as Thickener B.

In the succeeding examples two types of aging were carried out. These are referred to as regular and wrapped aging. The regular aging was 45 accomplished simply by treating the piece in a steam ager. In the wrapped ageing, the print was first rolled around a rod of approximately ½ inch diameter, the rod removed without unwinding and the roll wrapped in a piece of white cotton cloth which was wider than the print piece. The overlapping ends were tucked in and the print rolled in a second piece of cloth to make certain that there was no possibility of steam attacking the printed color without first passing through 50 the wrapping. The wrapped roll was aged for about 10 minutes in a steam ager. Regular ageing of cotton fabrics was carried out for about five minutes and rayon for ten minutes. The effect of 55 wrapping the printed piece is to increase the ageing temperature, thereby more nearly simulating plant ageing conditions.

*Example 3*

60 5 parts of dispersible Vat Scarlet 2GHN powder, a mixture of Hydron Orange powder (Color Index 1217) and Hydron Pink powder (6-6' dichloro 4,4' dimethyl 2-2' bis thionaphthene indigo), prepared according to United States Re-issue Patent 21,402 and containing about 1.8 parts 65 of real dye were blended with 1 part of the reaction product obtained by refluxing 60 parts of urea and 150 parts of normal butanol until the odor of ammonia practically disappeared. To 70 this was added 94 parts of Thickener A and the whole thoroughly mixed to produce a printing 75

color paste. A second paste was prepared from 5 parts of the same Vat Scarlet 2GHN with 95 parts of Thickener A. Both pastes were printed on samples of titanium dioxide pigmented viscose rayon flat crepe. The printed pieces were dried in a hot air oven, aged, both open and wrapped, at about 104° C., oxidized, soaped at the boil for five minutes with a 0.1% soap solution, rinsed and ironed dry. The prints from the paste containing the butyl carbamate were noticeably stronger and brighter than those obtained from the pastes containing the color only.

*Example 4*

One mol. portion of urea and two mol. portions of ethyl butanol were refluxed for about 14 hours until the ammoniacal odor given off by the reaction had practically disappeared. The reaction product, ethyl butyl carbamate, was isolated and used in duplicating the procedure of Example 3. The prints obtained from the paste containing the carbamate were noticeably stronger than those obtained from the paste containing color only.

*Example 5*

Additional portions of the two printing pastes of Example 3 were prepared and a third portion was prepared in which five parts of diethylene glycol was used to replace the five parts of butyl carbamate. These samples were allowed to stand at room temperature in covered vessels and the printing procedures of Example 3 were repeated at periodic intervals for several weeks. Comparison of the prints showed that the color yields obtained from the pastes containing the carbamate, when tested periodically, decreased only slowly whereas those from the other samples decreased rapidly. The decrease was most noticeable in the case of the glycol-containing paste.

*Example 6*

5 parts of a dispersible Golden Orange G powder (Color Index 1096), prepared according to U. S. Reissue Patent 21,402 and containing about 1 part of real dye, were made into a paste with 5 parts of water and 90 parts of Thickener B. A second 5 parts of Golden Orange R powder was pasted with 5 parts of a 6% dispersion of butyl carbamate and 90 parts of Thickener B. Each of these pastes were printed on titanium dioxide pigmented viscose rayon flat crepe and on 80 x 80 bleached unmercerized cotton print cloth. The printed pieces were air dried, aged at about 104° C. in a steamager both regularly and wrapped. After ageing the pieces were oxidized, soaped, rinsed and dried. The prints obtained from the pastes containing the butyl carbamate were approximately 10% stronger than those prepared from the other sample.

*Example 7*

The procedure of Example 6 was duplicated except that 5 parts of a dispersible Dark Blue BO powder (Color Index 1099), prepared according to U. S. Reissue Patent 21,402 and containing approximately 2 parts of real dye were used in place of the Golden Orange G. Prints from the paste containing the carbamate were distinctly stronger than from the pastes containing only color.

*Example 8*

The procedure of Example 6 was repeated, replacing the Golden Orange G with 5 parts of a dispersible Hydron Orange R powder (Color Index 1217) and containing 1.2 parts of real dye.

Again the prints obtained from the paste containing the butyl carbamate were much stronger both on pigmented rayon and cotton pieces than those obtained from the paste in which no printing assistant was used.

*Example 9*

A sample of Hydron Orange R wet presscake was dispersed with the sodium salt of disulfodinaphthylmethane and adjusted with water to contain approximately 12% real color. 10 parts of this slurry was pasted with 10 parts of water and 80 parts of Thickener B. A second 10 parts of the printing color was mixed with 5 parts of water and 5 parts of a 6% dispersion of butyl carbamate and 80 parts of Thickener B. A third 10 parts of color was mixed with 10 parts of a 6% solution of butyl carbamate in alcohol and 80 parts of Thickener B. Each of these pastes were printed on titanium dioxide pigmented, viscose rayon and 80 x 80 bleached, unmercerized cotton. Again the use of the printing assistant both as a slurry and as an alcohol solution gave definitely stronger color yields than when no assistant was used.

*Example 10*

1 mol portion of urea and 2 mol portions of octyl alcohol were refluxed until the ammoniacal odor given off by the reaction had disappeared. The reaction product was isolated and substituted for the butyl carbamate of Example 9. Example 9 was repeated with this change. Again the use of the carbamate printing assistant both as slurry and as an alcohol solution gave definitely improved color yields.

*Example 11*

Example 9 was again repeated making use of the reaction product of ethyl alcohol and phenyl nitrourea as a printing assistant. Again the presence of the carbamate in the printing paste was found to yield prints which were definitely stronger, the improvement being particularly noticeable on rayon.

We claim:

1. A color composition comprising a vat dye and a crystallizable alkyl carbamate having the structural formula:



in which R is a member selected from the group consisting of the primary and secondary alkyl radicals of from 3-12 carbon atoms, and R<sub>1</sub> and R<sub>2</sub> are members selected from the group consisting of hydrogen and the alkyl radicals of from 1-4 carbon atoms, R<sub>1</sub> and R<sub>2</sub> being identical when both are alkyl radicals.

2. A color composition comprising a vat dye and a crystallizable alkyl carbamate of the formula



in which R is a member selected from the group consisting of the primary and secondary alkyl radicals of from 4-8 carbon atoms.

3. A color composition according to claim 2 in which R is the n-butyl radical.

4. A color composition according to claim 2 in which R is an ethyl butyl radical.

5. A color composition according to claim 2 in which R is an octyl radical.

6. A dye powder composition comprising a vat

dye and a crystalline alkyl carbamate of the formula



in which R is a member selected from the group consisting of the primary and secondary alkyl radicals of from 4-8 carbon atoms.

7. A dye powder composition according to claim 6 in which R is the n-butyl radical.

8. A dye powder composition according to claim 6 in which R is an ethyl butyl radical.

9. A dye powder composition according to claim 6 in which R is an octyl radical.

10. A printing paste composition comprising a vat dye, a thickener and a crystallizable alkyl carbamate of the formula



in which R is a member selected from the group consisting of the primary and secondary alkyl radicals of from 4-8 carbon atoms.

11. A printing paste composition comprising a highly dispersed vat dye, a thickener and a printing assistant comprising a crystallizable alkyl carbamate of the formula



in which R is a member selected from the group consisting of the primary and secondary alkyl radicals of from 4-8 carbon atoms, said paste being prepared by compounding a vat dye powder of high autodispersibility and the printing assistant with the thickener.

12. A method of printing with vat colors which comprises printing a fabric with a printing paste composition comprising a vat dye, a thickener and a crystallizable alkyl carbamate of the formula



in which R is a member selected from the group consisting of the primary and secondary alkyl radicals of from 4-8 carbon atoms.

ROY HERMAN KIENLE,  
CHESTER ALBERT AMICK.

#### REFERENCES CITED

The following references are of record in the file of this patent:

#### UNITED STATES PATENTS

| Number    | Name          | Date          |
|-----------|---------------|---------------|
| 2,143,490 | Meyer         | Jan. 10, 1939 |
| 2,047,069 | Hentrich      | July 7, 1936  |
| 2,116,521 | Kritchevsky   | May 10, 1938  |
| 1,964,564 | Ulrich        | June 26, 1934 |
| 1,933,945 | Ulrich        | Nov. 7, 1933  |
| 2,184,495 | Graenecker    | Dec. 26, 1939 |
| 2,117,623 | Paquin et al. | May 17, 1938  |
| 1,856,434 | Schmidt       | May 3, 1932   |
| 2,090,511 | Crossley      | Aug. 17, 1937 |

#### FOREIGN PATENTS

| Number  | Country     | Date          |
|---------|-------------|---------------|
| 156,726 | Switzerland | Feb. 16, 1933 |
| 514,738 | Germany     | Dec. 17, 1930 |